

# United States Patent Office

3,252,412

Patented May 24, 1966

1

3,252,412

## PROCESS FOR PRODUCING HECTOGRAPHIC PRINTS

Albert Emiel Van Hoof, Berchem-Antwerp, Belgium, assignor to Gevaert Photo-Producten N.V., Mortsel-Antwerp, Belgium, a company of Belgium

No Drawing. Filed Oct. 7, 1960, Ser. No. 61,052

Claims priority, application Netherlands, Oct. 8, 1959, 244,134

13 Claims. (Cl. 101—149.4)

The present invention relates to the manufacture of a number of hectographic prints from a photographically obtained matrix.

It is known from the British specification 804,076 (U.S. Serial No. 582,944, filed May 7, 1956, and now abandoned) to obtain tens of prints from any original whatever by making a photographic reproduction of the original on light-sensitive material provided with a silver halide emulsion which contains a preferably at most slightly colored and at most slightly water-soluble color coupler, wherein by tanning development the formed image is caused to adhere selectively to the support of the photographic material, while the rest of the emulsion is removed, by bringing the remaining tanned image, containing the color coupler, in the presence of a print liquid into contact as master sheet with a print paper the print paper and/or print liquid containing means for converting the color coupler into dyestuff and/or to dissolve the formed dyestuff or the color coupler, and by bringing again and again new print paper into contact with the matrix in the presence of print liquid.

In said British specification (U.S. Serial No. 582,944, filed May 7, 1956) as well as in U.S. patent application Serial No. 37,101, filed June 20, 1960, now Patent No. 3,129,097, several methods of embodiment are described for the manufacture of this matrix or relief image.

According to the examples of said British specification (U.S. Serial No. 582,944, filed May 7, 1956) the paper on which is to be printed and/or the print liquid must contain a means for converting the color coupler into dyestuff very rapidly and at room temperature. If the emulsion contains a leucobase, an oxidizing agent must be present in the paper and/or in the print liquid. For this purpose, multivalent cerium-, vanadium-, manganese compounds, dichromates etc. are of particular importance. Further, the layer of the print paper can contain products such as heteropoly acids which increase the light-fastness of the organic dyestuff.

Finally, the print liquid must be used in such a way that either the color coupler in the emulsion or the formed dyestuff be dissolved and can diffuse to the print paper.

An aqueous solution of an acid, preferably an organic acid such as oxalic acid, citric acid, tartaric acid etc. is particularly suited as print liquid when leucobases are used.

In Example 3 of said British specification (U.S. Serial No. 582,944, filed May 7, 1956) a method is described wherein a gelatin relief, containing both a leucobase and an oxidizing agent, is brought into contact with ordinary paper in the presence of an aqueous acid solution whereby simultaneously the leucobase is converted into the dyestuff, the latter diffuses over to the paper and gives there-in a colored print of the original.

Bringing the matrix into contact with the paper can occur in a printing apparatus of the alcohol duplicator type. If in this process an aqueous acid solution is used as print liquid, there is the risk that the construction material of the duplicator is affected. Moreover, the paper moistened with aqueous solution remains easily sticked to the image relief serving as matrix.

In order to avoid all these drawbacks, the leucobase can first be converted into a dyestuff after obtaining the

2

image relief containing said leucobase of a triphenyl methane dyestuff, by one or more bath treatments with an oxidizing agent and a diluted acid and by making thereafter prints in an ordinary alcohol duplicator by means of the ordinary alcohol duplicator print liquid which in most cases contains one or more lower aliphatic alcohols.

The disadvantage of this method, however, is to be found in the rinsing out of the formed dyestuff during the treatment which is necessary for the conversion of the leucobase into dyestuff so that only a small number of rather unsharp prints is obtained.

It has now been found that a large number of sharp prints can be obtained from an original by using the method of said British specification (U.S. Serial No. 582,944, filed May 7, 1956) by treating the formed relief image with an oxidizing agent, an acid and a precipitating agent for the dyestuff formed by oxidation before printing by means of the alcoholic print liquid.

The new process offers the important advantage that the use of acid solutions in the alcohol duplicator is omitted avoiding in this way the corroding action on metal parts.

Another important advantage consists therein that the dissolution of the color coupler in the acid bath is considerably counteracted in this way.

As suitable oxidizing agents which can be applied in the new process multivalent cerium-, vanadium- and manganese compounds, dichromates etc. are mainly considered.

As suitable acids which can be applied in the new process mineral acids such as phosphoric acid, nitric acid, sulfuric acid, and organic acids, such as acetic acid, citric acid, glycolic acid, sulfamic acid and tartaric acid, are mainly considered.

As precipitating agents for the dyestuffs formed by oxidation which do not or at least little solubilize the latter in aqueous treating baths, those can be chosen which are used for manufacturing pigments and for mordanting basic dyestuffs on textile fibers. Some of the most appropriate representatives are some iso- or hetero-poly acids and their salts, such as alkali- and ammonium molybdates, -tungstates, phosphomolybdates, phosphotungstates, silicotungstates, phosphomolybdate-tungstates etc. In this respect also some organic acids such as dichloro acetic acid, trichloro acetic acid and sulfosalicylic acid offer interesting possibilities for application.

In principle, the treatment of the washed image relief according to the method of the present invention is carried out in several steps. Thus, the master sheet can first be led through an oxidizing bath consisting of a diluted aqueous potassium permanganate solution and next through an acid bath consisting of an aqueous diluted acid wherein the precipitating agent is dissolved for the triphenyl methane dyestuff formed by oxidation. This precipitating agent, however, can also be dissolved in the oxidizing bath.

Another embodiment of the process according to the present invention consists therein that the washed image relief after treatment with an oxidizing agent is immersed in an acid solution the acid of which serves itself as precipitating agent of the dyestuff such as for instance trichloroacetic acid.

A further and particular simple embodiment of the process according to the present invention consists therein that the washed image relief is treated with only one solution which besides the oxidizing agent also contains a precipitating acid. Instead of an acid which serves as precipitating agent for the dyestuff, also a combination of a non-precipitating acid and a precipitating agent can be chosen. Evidently, the acid must at least for some time be compatible with the oxidizing agent.

After this treatment the obtained master sheet can be

used, after removal of the excess of liquid, for manufacturing some tens of prints onto paper which was moistened with a print liquid mainly consisting of a lower aliphatic alcohol such as methanol, ethanol or isopropanol or of a mixture of such alcohols either mutually or with water. This print liquid can evidently also contain the usual ingredients for composing duplicator liquids. Such compositions are i.a. described in J. Chem. Education, 32, 200-202 (1955) and in the American patent specifications 2,228,108, 2,262,488 and 2,294,711.

The following examples illustrate the invention without limiting, however, the scope thereof.

#### Example 1

A material manufactured as described in British specification No. 804,076 (U.S. Serial No. 582,944, filed May 7, 1956) is reflectographically exposed through an original. After hardening development according to the above U.S. application Serial No. 37,101, filed June 20, 1960, the non-developed and consequently non-tanned parts of the gelatin emulsion layer are washed away. The image relief thus obtained is immersed for 5 seconds in a 1% aqueous potassium permanganate solution whereafter the excess of solution is removed by squeezing between two rubber rollers. This image relief is then immersed for 5 seconds into a 1% aqueous trichloroacetic acid solution. The excess of liquid is then removed by squeezing between two rollers whereafter the master sheet obtained is fixed on a duplicator containing isopropanol as print liquid. With this master sheet tens of sharp prints of the original to be reproduced are obtained.

#### Example 2

A gelatin relief image obtained as in Example 1 is immersed for 5 seconds in a 1% aqueous potassium permanganate solution whereafter the excess of solution is removed as in Example 1. This image relief is then immersed for 5 seconds in a 10% aqueous trichloroacetic acid solution and further treated as in Example 1 but printed in an alcohol duplicator containing isopropanol. Tens of sharp prints of the original to be reproduced are obtained.

#### Example 3

A gelatin relief image obtained and soaked with a potassium permanganate solution as in the foregoing example but containing leuco crystal violet instead of leuco malachite green, is immersed for 15 seconds, after removal of the excess of solution with blotting paper, in a solution of the following composition:

|                                 | Cm. <sup>3</sup> |
|---------------------------------|------------------|
| 20% aqueous citric acid         | 50               |
| 10% aqueous silicotungstic acid | 5                |

Further treatment as in Example 1 and printing with a print liquid of the following composition: ethanol 80%, 55 methanol 18% and methyl glycol 2%. Tens of sharp prints of the original are obtained.

#### Example 4

A gelatin relief image obtained as in Example 3 is immersed for 15 seconds in a 2.5% aqueous ammonium dichromate solution. After removal of the excess of solution, the relief image is immersed for 15 seconds into a solution consisting of:

|                                 | Cm. <sup>3</sup> |
|---------------------------------|------------------|
| 20% aqueous tartaric acid       | 50               |
| 10% aqueous silicotungstic acid | 3                |

Further treatment and printing as in Example 1 gives tens of sharp prints of the original.

#### Example 5

A gelatin relief image is obtained and soaked with a potassium permanganate solution as in Example 3 and the excess of liquid is removed by squeezing between two

rubber rollers. Next, the relief image is immersed into a solution of the following composition:

|                                     | Cm. <sup>3</sup> |
|-------------------------------------|------------------|
| 20% aqueous tartaric acid           | 50               |
| 10% aqueous sodium phosphomolybdate | 5                |

Further treatment and printing as in Example 2 gives tens of sharp prints of the original.

#### Example 6

10 A gelatin relief image obtained as described in Example 3 is immersed for 5 seconds into a solution of the following composition:

|                                   | Cm. <sup>3</sup> |
|-----------------------------------|------------------|
| 3% aqueous potassium permanganate | 40               |
| Glacial acetic acid               | 40               |

15 After removal of the excess of liquid by squeezing between two rubber rollers, tens of prints of the original are obtained as in Example 3.

#### Example 7

20 A gelatin relief image obtained as in Example 1 is immersed for 30 seconds into a solution of the following composition:

|                                   | Cm. <sup>3</sup> |
|-----------------------------------|------------------|
| 10% aqueous ammonium dichromate   | 4                |
| 20% aqueous trichloro acetic acid | 50               |

25 Further treatment as in Example 3.

#### Example 8

30 A gelatin relief image obtained as in Example 1 is immersed for 3 seconds into a mixture consisting of 20 cm.<sup>3</sup> of 20% aqueous trichloroacetic acid and 50 cm.<sup>3</sup> of a solution of the following composition

|                                              |     |
|----------------------------------------------|-----|
| Cerium (IV)-sulfate, g.                      | 41  |
| Concentrated sulfuric acid, cm. <sup>3</sup> | 28  |
| Water, cm. <sup>3</sup>                      | 500 |

35 Further treatment as in Example 3.

#### Example 9

40 A gelatin relief image obtained as in Example 1 is immersed for 15 seconds into a solution of the following composition:

|                                   | Cm. <sup>3</sup> |
|-----------------------------------|------------------|
| 3% aqueous potassium permanganate | 40               |
| Glacial acetic acid               | 40               |
| 10% aqueous ammonium molybdate    | 40               |

45 Further treatment as in Example 3.

I claim:

1. In a method of making multiple prints of a printing master in a spirit duplication process wherein:
  - (A) Said master is prepared by the steps of
    - (1) Exposing to an indicia-bearing original to be copied a light-sensitive photographic material including a support bearing a silver halide emulsion layer containing a finely-divided, water-insoluble, potential color-forming leuco-base of a triphenylmethane dyestuff,
    - (2) Subjecting the exposed photographic material to tanning development to form in said emulsion layer a positive latent mirror image of said original and harden the areas of said layer bearing said latent mirror image,
    - (3) Removing the unhardened areas of said layer to leave a positive relief mirror image of hardened emulsion attached to said support, and
    - (4) Subjecting the material from step (3) to oxidation and acidification to convert said leuco-base to a colored dyestuff; and
  - (B) Prints are made from said master resulting from
    - (A) by pressing into contact therewith print paper

moistened with an alcoholic print liquid comprising essentially an alcohol selected from the group consisting of methanol, ethanol, isopropanol and their mixtures; in combination, the improvement of contacting the positive relief mirror image prior to said print-making step (B) with an aqueous solution of a basic dyestuff mordanting agent to precipitate the colored dyestuff in the hardened areas of said emulsion layer.

2. The method of claim 1 wherein said relief image is contacted with said solution of said mordanting agent by immersing the image in said solution for a time of about 3-30 seconds and thereafter removing excess solution therefrom.

3. The method of claim 1 wherein said positive relief mirror image is contacted with an aqueous solution of a material selected from the group consisting of the isopoly acids, the heteropoly acids, and their alkali and ammonium salts.

4. The method of claim 1 wherein said material from step 3 is acidified by treatment with an aqueous solution of a weak organic acid.

5. The method of claim 1 wherein said triphenylmethane dyestuff is malachite green.

6. The method of claim 1 wherein said triphenylmethane dyestuff is crystal violet.

7. The method of claim 1 wherein said leuco-base of said dyestuff is oxidized by treatment with an aqueous solution of potassium permanganate.

8. The method of claim 1 wherein said leucobase of said dyestuff is oxidized by treatment with an aqueous solution of ammonium bichromate.

9. The method of claim 1 wherein said leucobase of said dyestuff is oxidized by treatment with an aqueous solution of cerium (IV) sulfate.

10. The method of claim 1 wherein said colored dyestuff is precipitated by treatment with an aqueous solu-

tion of a material selected from the group consisting of molybdcic acid and tungstic acid, the complexes of such acids with phosphorus and silicon, and the alkali metal and ammonium salts of said acids and said complexes.

5 11. The method of claim 10 wherein said material is molybdcic acid.

12. The method of claim 10 wherein said material is tungstic acid.

13. The method of claim 1 wherein said acidification and precipitation are effected simultaneously by treatment of said relief image with an aqueous solution of a material of the group consisting of dichloroacetic acid, trichloroacetic acid and sulfosalicylic acid.

#### References Cited by the Examiner

##### UNITED STATES PATENTS

|           |         |                   |       |           |
|-----------|---------|-------------------|-------|-----------|
| 1,923,625 | 8/1933  | Jackson           | ----- | 101-149.4 |
| 1,935,477 | 11/1933 | Martinez          | ----- | 90-93     |
| 2,034,220 | 3/1936  | Allison           | ----- | 96-72     |
| 2,054,261 | 9/1936  | Lierg             | ----- | 96-35     |
| 2,266,456 | 12/1941 | Wilder            | ----- | 96-21 X   |
| 2,855,300 | 10/1958 | Chalkley          | ----- | 96-90 X   |
| 2,898,852 | 8/1959  | Staeble et al.    | ----- | 96-28     |
| 3,049,994 | 8/1962  | Raczynski et al.  | ----  | 101-149.5 |
| 3,096,711 | 7/1963  | Ritzerfeld et al. | ----  | 101-149.4 |
| 3,152,898 | 10/1964 | Hepher            | ----- | 96-33 X   |

##### FOREIGN PATENTS

539,781 9/1941 Great Britain.

##### OTHER REFERENCES

Glafkides, "Photographic Chemistry," 1960, vol. 2, Fountain Press, London, page 713.

35 ALEXANDER D. RICCI, Primary Examiner.

MILTON STERMAN, Examiner.